

## UNITED STATES PATENT OFFICE

GRIGORI PETROFF, OF MOSCOW, RUSSIA

## PROCESS FOR OBTAINING SOAP

No Drawing. Application filed January 16, 1926, Serial No. 81,833, and in Germany December 21, 1925.

This invention relates to processes of preparing hard soaps and soap powders from vegetable and animal fats in the nature of drying and semi-drying oils, and it comprises 5 a process in which such oils, prior to saponification with alkalies in the usual way, are treated with water-insoluble salts of chromic acid in the presence of an acid other than chromic acid which is capable of forming 10 water insoluble salts with the metallic radical of the chromate used.

Many drying and semi-drying oils are totally unsuited for soap making purposes due to the fact that these oils, on saponification in the usual way, yield soft or liquid 15 soaps. In the arts, hard soaps, such as those made by saponifying solid fats which on saponification yield salts of stearic acid and other fatty and non-drying acids, capable of 20 forming hard soaps, are more desirable. Soft soaps have but limited utility because of their physical nature.

It is an object of this invention to so treat 25 drying and semi-drying oils such as linseed, sunflower, cottonseed oil, etc., that these oils, normally unsuitable for soap making, may be converted into substances which, on saponification in the usual way, are capable of giving 30 hard soaps and soap powders. Without the preliminary treatment I have discovered, such drying and semi-drying oils, as is well known, yield greasy and smeary soaps unfit 35 for consumption.

I have discovered that these drying oils 40 may be made to give hard soaps on saponification if, preliminary to the saponification step, the oils are subjected to the action of a water insoluble chromate, in the presence of an acid other than chromic capable of precipitating 45 water insoluble salts with the metallic radical of the chromate salt used. As chromates, I may advantageously use calcium, barium or lead chromate; and as the precipitating acid, I find suitable sulfuric, phosphoric or other acids yielding insoluble salts of calcium, 50 barium or lead.

In general, the drying or semi-drying oils are treated with an insoluble chromate and a precipitating mineral acid, such as sulfuric 55 and phosphoric and the resulting mixture al-

lowed to stand for a few hours. The mixture stratifies and the bottom layer, which consists of an aqueous solution of the mineral acid and the insoluble salt of this acid, is drawn off. The oil layer is washed with water and thereafter saponified in the usual way. 55

In saponifying the treated oil, the washed oil is either boiled or simply mixed in the cold with an aqueous alkali solution in such quantity that all the fatty acids contained in 60 the oil (which may in part be in the form of glycerides) are neutralized, that is, converted into alkali metal salts. The saponification step is the usual one employed in soap 65 making.

As a specific example of an advantageous 70 way of carrying out my process, I introduce into a closed vessel or tank 100 parts of sunflower oil, 2 parts of barium chromate, 5 parts of 30 per cent sulfuric acid and 30 parts 75 of water. These materials are mixed in the cold, or at ordinary temperature (10° to 30° C.) and allowed to stand over a period of 10 to 15 hours. The bottom layer, the mixture having stratified, is drawn off and the 80 oil layer washed with water. The bottom layer consists of dilute sulfuric acid and settled barium sulphate. The oil layer consists of sunflower oil which presumably has been oxidized to some extent, since sunflower oil, 85 in common with other drying and semi-drying oils, is unsaturated. The exact phenomena occurring however is not clear. I content myself with noting the fact that drying and semi-drying oils, when subjected to 90 the above treatment, give hard soaps on saponification.

The so prepared washed oil is then saponified with 50 parts of a 30 per cent solution of caustic soda. This saponification step is well 95 known in the art and may be carried out in the usual way, either in the cold or at an elevated temperature.

I have further found that hard soaps so prepared from drying and semi-drying oils 100 are improved if to the soap, or during saponification of the oils, a small quantity of a powdered metal is added. The amount to be added is only that required to prevent the darkening of the soap on standing. One-

tenth of one per cent based on the soap is usually sufficient and powdered zinc and aluminum are advantageously used. These metals act to inhibit any oxidation of the soap on exposure to atmospheric influences.

5 Various fillers may be added to the soap, such as finely divided clay, cellulose, etc. as is customary.

What I claim is:

- 10 1. In the process of preparing hard soaps from drying and semi-drying oils, the step which comprises treating the oil with a water insoluble metallic chromate in the presence of a mineral acid other than chromic 15 capable of forming water insoluble salts with the metallic radical of the chromate used.
- 20 2. In the process of preparing hard soaps from drying and semi-drying oils, the step which comprises treating the oil with an alkaline earth metal chromate in the presence of a mineral acid other than chromic capable 25 of forming water insoluble salts with the alkaline earth metal.
- 30 3. In the process of preparing hard soaps from drying and semi-drying oils, the step which comprises treating the oil with a water insoluble chromate in the presence of sulfuric acid.
- 35 4. In the process of preparing hard soaps from drying and semi-drying oils, the step which comprises treating the oil with barium chromate in the presence of sulfuric acid.
- 40 5. In the process of preparing hard soaps from drying and semi-drying oils, the steps which comprise treating the oil with an alkaline earth metal chromate in the presence of a mineral acid capable of forming water insoluble salts with the alkaline earth metals, allowing the mixture to stand, drawing off the stratified lower aqueous layer, and washing the oil.

In testimony whereof I have signed my name to this specification.

GRIGORI PETROFF.

45

50

55

60

65